

## UNITED STATES PATENT OFFICE

2,073,641

## LUBRICATING OILS

Leo Liberthson, New York, N. Y., assignor to L. Sonneborn Sons, Inc., a corporation of Delaware

No Drawing. Application October 2, 1934,  
Serial No. 746,514

5 Claims. (Cl. 87—9)

This invention relates to improved lubricating oils and a process of preparing same, and especially to lubricating oils having a low pour point and being substantially non-emulsifiable.

5 Lubricating oils, and especially lubricating oils containing wax or waxy hydrocarbons in solution tend to have a high pour point. In the case of lubricating oils containing wax or waxy hydrocarbons, the latter compounds have a tendency to precipitate when the oil is cooled, thereby causing the oil to set or gel, and causing the oil to flow sluggishly or not at all. Lubricating oil distillates derived entirely or principally from the distillation of so-called Pennsylvania crude oil belong generally to the waxy class mentioned.

10 It is known that the addition of small amounts of voltol (an oil which has been polymerized by the action of a silent electrical discharge) to a lubricating oil will lower the normal pour point of such oil. However, the presence of such voltol in lubricating oils is in many cases disadvantageous in one important respect, viz.; the tendency of such a mixture to permanently emulsify with water. When such a mixture is used in a lubricating oil in apparatus where it comes in contact with water, for example, in a turbine or in a crank-case, the mixture forms an emulsion with the water, which raises the pour point of the lubricant and gives poor lubrication.

15 This tendency to emulsify is due to the fact that voltol is in reality a blend of mineral and vegetable oil, such blend having been found to be infinitely more susceptible to polymerization by means of a silent electrical discharge than mineral oil alone. The mineral oil can be designated as the unsaponifiable component and the vegetable oil as the saponifiable component of the original voltol.

20 I have discovered that if the unsaponifiable component of voltol is isolated from the voltol, such component may be added to a lubricating oil to lower its pour point without the disadvantages attending the use of the original voltol. This may be understood from the behavior of the so modified oil by subjecting it to the well known "A. S. T. M." demulsibility test. In this test, steam is conducted into a definite amount of oil and permitted to condense for a definite period of time. The mixture of oil and condensate should then separate into two layers within a specified time of not more than ten minutes.

25 Two different types of voltol, differing only in the relative proportions of mineral oil to vegetable oil, were treated according to this inven-

tion; one a Belgian voltol sold under the trade name of "Electrion" and a second, German voltol, designated "End voltol". The physical characteristics of these two voltols are as follows:—

|                      | "Electrion"                     | "End voltol"                     | 5  |
|----------------------|---------------------------------|----------------------------------|----|
| Gravity              | 23.1 A. P. I.                   | 18.3 A. P. I.                    |    |
| Vis. Saybolt 210° F. | 733 sec.                        | 975 sec.                         |    |
| Pour test            | 40° F.                          | 15° F.                           |    |
| Flash point          | 410.                            | 400.                             | 10 |
| Fire point           | 465.                            | 445.                             |    |
| Color (Lovibond)     | 20 yellow 5 red $\frac{1}{2}$ " | 20 yellow 14 red $\frac{1}{2}$ " |    |
| Acidity              | 0.63 Mg KOH                     |                                  |    |
| Alkalinity           | 0.47.                           |                                  |    |
| Iodine value         | 35.2.                           | 17.8.                            |    |
| Saponification No.   | 74.7.                           | 10.0.                            |    |
| Ash                  | 0.039%                          |                                  | 15 |

20 Each of these voltols was treated according to the well known Spitz-Hoenig method, which consists in treating a mixture of mineral and vegetable oil with alkali to saponify the fat, adding sufficient 50% alcohol to dissolve the soap formed, adding a light petroleum solvent such as benzine, shaking and allowing the mass to separate into two layers, a bottom layer of aqueous alcoholic solution of soap and an upper layer of a benzine solution of mineral oil, from which mineral oil can be isolated by distilling off the benzine. In applying this method to the above voltols a mineral oil was obtained having the following characteristics:—

|                   |                      |    |
|-------------------|----------------------|----|
| Gravity           | 23.7 A. P. I.        |    |
| Vis. Say. 100° F. | 311 sec.             |    |
| Vis. Say. 210° F. | 55 sec.              |    |
| Flash point       | 400                  |    |
| Fire point        | 450                  | 35 |
| Color             | #3 $\frac{1}{4}$ NPA |    |
| Saponification    | #2.5                 |    |
| Iodine #          | 10.5                 |    |

25 When 1% of this unsaponifiable oil was added to a waxy lubricating oil of Pennsylvania origin, having a normal pour point of 25 to 30° F., the pour point of the mixture was lowered to —5° F. and demulsification (according to the A. S. T. M. demulsibility test) took place in about 30 seconds. 45 With original voltol and the above lubricating oil, the pour point of the mixture was also —5° F., but a permanent emulsion was formed when subjected to the A. S. T. M. test.

30 In the case of an oil containing wax or a waxy hydrocarbon, the amount of unsaponifiable constituent of voltol to be added will vary from 0.2 up to 10% of the total and will, in general, be sufficient to produce a reduction in pour test or pour point of from 10 to 50° F. Within these limits 55

the amount added has no appreciable influence on viscosity. For a reduction in pour test of about 15° F., say from 25 to 10° F., one-half of 1% is ordinarily sufficient; and for a reduction of 5 25° F., say from 25° to 0° F., 1% will ordinarily be sufficient.

Ordinary voltol and unsaponifiable voltol according to this invention were added to lubricating oils having the following characteristics:

10 An S. A. E. 40 blend of Pennsylvania residual and neutral oils having:

Specific gravity..... 28 A. P. I.  
Viscosity (Say.) at 210° F..... 79 sec.  
15 Flash point..... 450° F.  
Fire point..... 515° F.  
Color (Lovibond)..... 20 yellow 38 red 1/2  
Pour point..... 25° F.

When 0.5, 1, 5 and 10% of ordinary voltol were 20 added, the pour points of the mixtures were lowered to 10, -5, -10, and -10° F. respectively, the other factors remaining substantially the same. Demulsibility tests of the mixtures however were all above ten minutes. With the same 25 amounts of unsaponifiable voltol, the same lowering of the pour points resulted, but in each of the latter cases, demulsibility occurred in less than one minute.

A Pennsylvania distillate having:

30 Specific gravity..... 29 A. P. I.  
Viscosity (Say.) at 210°..... 200-205 sec.  
Flash point..... 420° F.  
Fire point..... 470° F.  
Pour point..... 30-35° F.

When 0.5, 1, 5 and 10% of ordinary voltol were 35 added, the pour points of the mixtures were lowered to 5, -5, -10 and -10° F. respectively, the other factors remaining substantially the same. Similar pour point depressing values were obtained with similar amounts of unsaponifiable 40 voltol. However, with ordinary voltol, demulsibility tests were over ten minutes, while with unsaponifiable voltol, demulsibility occurred in less 45 than one minute.

A Pennsylvania distillate having:

Specific gravity..... 30 A. P. I.  
Viscosity (Say.) at 210° F..... 145-150 sec.  
Flash point..... 405° F.  
50 Fire point..... 460° F.  
Pour point..... 10° F.

With 0.5, 1, 5 and 10% of ordinary voltol, the pour points of the mixtures were lowered to -5, 55 -15, -25 and -25° F. respectively, the other factors remaining substantially the same. Demulsibility tests of the mixtures in each case, however, were above ten minutes. With similar amounts of unsaponifiable voltol, similar lowering 60 of the pour points resulted, but in each case demulsibility occurred in less than one minute.

I have suspected that emulsification with ordinary voltol is due to the higher polymers resulting from the electrical treatment by which the 65 voltol is produced, and this suspicion is more or less confirmed by the presence of difficultly soluble matter which is found between the benzine and

alcoholic layers in the Spitz-Hoenig treatment. This matter is a yellow, gelatinous rubbery substance, difficultly soluble in oil, but sufficiently so to give a permanent emulsion when its solution in oil is mixed with water. However, I do not 5 wish to be limited to any theory as to the identity of the emulsifying agent or to the cause of emulsification of the ordinary voltol.

My invention includes all lubricating oils containing wax or crystallizable hydrocarbons, and 10 I claim broadly a lubricating oil having a normal pour point and containing the unsaponifiable constituent of voltol in amount and potency sufficient to reduce the normal pour point of the lubricating oil, the product having good demulsibility and substantially the same viscosity as the lubricating oil. By good demulsibility I mean a product which, when subjected to the A. S. T. M. demulsibility test, will separate into two well 15 defined layers in less than ten minutes. 20

I claim:

1. A product comprising a lubricating oil having a pour point caused by wax therein, and up to about 10% of the unsaponifiable constituent 25 of a polymerized oil of potency sufficient to appreciably reduce the normal pour point of said lubricating oil, said polymerized oil being prepared by the action of a silent electrical discharge, said product being substantially non-emulsifiable. 30

2. A product comprising a lubricating oil having a pour point caused by wax therein, and up to about 10% of the unsaponifiable constituent of a polymerized oil of potency sufficient to reduce the normal pour point of said lubricating oil at least 10° F., said polymerized oil being prepared by the action of a silent electrical discharge, said product being substantially non-emulsifiable. 35

3. A product comprising a lubricating oil having a pour point of at least 10° F. caused by wax therein, and up to about 10% of the unsaponifiable constituent of a polymerized oil of potency sufficient to reduce the normal pour point of said lubricating oil at least 10° F., said polymerized 40 oil being prepared by the action of a silent electrical discharge, said product being substantially non-emulsifiable. 45

4. A product comprising a petroleum lubricating oil distillate having a pour point caused by 50 wax therein, and up to about 10% of the unsaponifiable constituent of a polymerized oil of potency sufficient to appreciably reduce the normal pour point of said distillate, said polymerized oil being prepared by the action of a silent electrical discharge, said product being substantially non-emulsifiable. 55

5. A product comprising a petroleum lubricating oil distillate having a pour point of at least 10° F. caused by wax therein, and up to about 60 10% of the unsaponifiable constituent of a polymerized oil of potency sufficient to reduce the normal pour point of said distillate at least 10° F., said polymerized oil being prepared by the action of a silent electrical discharge, said product being substantially non-emulsifiable. 65

LEO LIBERTHSON.